

Feb. 23, 1943.

R. S. MORSE

2,311,681

PREPARATION OF IMPROVED PAINT OILS

Filed April 9, 1940



RICHARD S. MORSE

INVENTOR

*Newton M. Penrose*  
BY *Warren H. Cannon*

ATTORNEYS

## UNITED STATES PATENT OFFICE

2,311,681

## PREPARATION OF IMPROVED PAINT OILS

Richard S. Morse, Rochester, N. Y., assignor to  
Distillation Products, Inc., Rochester, N. Y., a  
corporation of Delaware

Application April 9, 1940, Serial No. 328,701

8 Claims. (Cl. 202—52)

This invention relates to a method for preparing improved bodied or drying oils satisfactory for use in paints and the like.

It is known in the art to prepare thickened oils by subjecting drying or semi-drying oils and the like to bodying or polymerization treatment. Numerous methods are known in the art but, in general, they comprise heating or oxidation or combinations of the two. Oxidized oils are generally made by blowing air through the oil at an elevated temperature. Such oils are known as blown oils. This procedure is usually applied to cheaper oils and yields a relatively inferior product. The heating procedure is usually applied to better grade oils and yields a better product. The oil is usually heated in a vacuum or in the presence of an inert gas such as nitrogen or carbon dioxide.

In Oosterhof Patent 2,065,728 it is proposed that such polymerized or bodied oils be subjected to high vacuum unobstructed path distillation to remove nonpolymers. The procedure involved the removal of relatively large amounts of nonpolymers running from 20-30% and above. The residue was shown to have improved qualities such as drying time. The removal of such large amounts results in an undistilled residue having high viscosity which tends to form a hard film on the vaporizing surface giving rise to decomposition and charring during the distillation. Other difficulties are encountered.

This invention has for its object to provide a simple and economical method for removing non-polymerized materials from a bodied oil. Another object is to provide a method for preparing a good quality drying oil by distillation of bodied oils which will avoid the difficulty of removal of large amounts of non-polymers. A still further object is to provide a process which will avoid the above described difficulties, namely, clogging and charring of the still. Another object is to provide a method for removing non-polymers which is economical and substantially simplified. Other objects will appear hereinafter.

These and other objects are accomplished in accordance with my invention which includes subjecting the bodied or polymerized oil to high vacuum unobstructed path distillation and removing only about 2-12% of non-polymerizable and the like as distillate. I have discovered that the removal of as little as 2% as distillate yields a drying oil of vastly improved qualities and that the removal of more than 12% has no beneficial effects. In other words, the maximum quality is obtained by removal of about 10% non-poly-

merizable or volatile and the removal of more than 12% is not attended by an increase in desirable properties, such as drying time, film hardness, water-resistance, etc. For instance, I have found that when my invention is applied to bodied menhaden oil the removal of as little as 2% as distillate yields an undistilled residue which has as fast a drying time as linseed oil. This represents a remarkable advance since it is well known that drying oils heretofore prepared from the fish oils have been far inferior to linseed oil.

My invention is applicable to the distillation of bodied oils prepared by any of the above described bodying treatments or by conventional bodying treatments known in the art. The process is applicable to bodied oils which are bodied in any particular degree. It is applicable to bodied vegetable and marine animal oils, such as bodied linseed, soy, oiticica, walnut, sardine, salmon, menhaden, etc. oils. In the case of marine animal oils, it is desirable that the bodied oil be prepared from one which has an iodine number of approximately 120 or above.

The bodied oil is subjected to distillation under high vacuum unobstructed path distillation conditions. Such distillations are well known in the art. The pressure is usually below 2 mm. and is preferably below .1 mm., such as .01 to .001 mm. The temperature of distillation will vary with the particular oil treated and the distillation conditions. Temperatures of 150-300° C. are generally used. Higher or lower temperatures are usable but are not commercially satisfactory because of decomposition or slow rate of distillation. Temperatures of about 175-275° C. are preferred.

Although it is perfectly satisfactory to employ an ordinary high vacuum unobstructed path still in which the bodied oil is flowed over the vaporizing surface in a thin film by gravitational force, I much prefer to use centrifugal distillation apparatus in which the bodied oil is caused to flow over the heated vaporizing surface by forces greater than gravity. In one form of apparatus for such distillation the bodied oil is introduced onto the center of a heated rapidly rotating disc. It is caused to flow thereover in an exceedingly thin film by centrifugal force. Undistilled residue is removed from the disc at its periphery. The disc is maintained under a high vacuum and volatiles given off are condensed upon a condensing surface separated from the disc by unobstructed space. Stills of this type enable the use of temperatures in the lower portion of the foregoing range. They also enable a high rate

of distillation and avoid thermal decomposition. Such stills are disclosed in detail in Hickman application 99,632 filed September 5, 1936, now Patent No. 2,210,927 dated August 13, 1940.

Regardless of the type of still used, which may be a batch still in which the distillant is separated from the condensing surface by unobstructed space, the distillation is adjusted as to time and temperature so that approximately 2-12% of distillate is removed. The distillate is withdrawn from the still and will be found to consist of materials which are substantially non-polymerizable and which apparently inhibit polymerization in the original oil. The 2-12% distillate contains a mixture of complex substances which comprise among other compounds free fatty acids, sterols, hydrocarbons, decomposition products, and non-polymerizable glycerides. The undistilled residue is withdrawn from the still preferably after cooling and will be found to be a drying oil of high quality.

By the elimination of 2-12% distillate a maximum improvement in drying time and hardness is achieved. There appears to be no additional advantage to be obtained by the removal of further volatile material. This treatment reduces the drying time to approximately 50% of the original bodied oil and the hardness, water resistance, etc., are likewise improved.

In the accompanying drawing to which reference is made, I have illustrated the manner in which the drying properties of bodied oils are improved by removal of volatile components therefrom. This is shown by the curve in which percent distillate removed is plotted against drying time of residue. The notation at 130 represents the drying time of linseed oil. It is seen that the removal of as little as 2% distillate results in a residue having a drying time equal to that of linseed oil. Since this particular curve was determined by experiments on bodied menhaden oil, it well illustrates the remarkable improvement in drying qualities obtained by my invention. The results with other oils are much the same. The curve also illustrates the fact that in the neighborhood of 10-12% there is a critical change and that thereafter no advantage is to be obtained in drying qualities by removal of additional volatile matter.

#### Example

A heavy bodied menhaden oil having the following characteristics:

|                           |                  |    |
|---------------------------|------------------|----|
| Acid value                | 3.78             | 55 |
| Refractive index          | 1.4840 at 40° C. |    |
| Viscosity—poises          | 10.5 at 25° C.   |    |
| Iodine value              | 112.0            |    |
| Per cent non-saponifiable | 3.85             |    |
| Sap. number               | 222.0            | 60 |

was subjected to high vacuum unobstructed path distillation by causing it to flow in a thin film over a rotating plate of a centrifugal still having a diameter of 14 inches. The plate was maintained at a temperature of 180°. The pressure was approximately .001 mm. A 10% fraction was distilled off which was found to be components of lower molecular weight, mainly free fatty acids and non-saponifiable matter. The undistilled residue was removed, cooled to room temperature, and mixed with a drier, such as .5% lead in the form of lead naphthenate, .05% manganese in the form of manganese naphthenate, and .05% cobalt in the form of

75 cobalt naphthenate. The bodied oil-drier mixture was then spread on glass in a thin film of approximately .001 inch thickness. The film was maintained at room temperature and humidity. A finger smear test was made every 15 minutes. It was found that the residue had dried to complete hardness in 80 minutes. The drying time of the original material before distillation was 150 minutes.

10 In a companion distillation the same oil was treated to remove 30% distillate. The residue was then tested in the same way. It was found that the drying time was substantially the same as that of the residue from which only 10% was removed.

15 What I claim and desire to be secured by Letters Patent of the United States is:

1. The process of producing an improved drying oil which comprises in combination subjecting a bodied drying or semi-drying vegetable or animal oil to high vacuum, unobstructed path distillation until not more than about 12% of said bodied vegetable or animal oil has been distilled and then removing the undistilled portion of the bodied oil from the still as the improved drying oil.

2. The process of producing an improved drying oil which comprises in combination subjecting a bodied vegetable or animal oil which vegetable or animal oil in its unbodied condition had an iodine number above about 120, to high vacuum unobstructed path distillation until not more than about 12% of the bodied vegetable or animal oil has been distilled, and then removing the undistilled portion of the bodied oil from the still as the improved drying oil.

3. The process of producing an improved drying oil which comprises in combination subjecting a bodied fish oil, which fish oil in its unbodied condition had an iodine number above about 120, to high vacuum unobstructed path distillation until approximately 2-12% of the bodied fish oil has been distilled, and then removing the undistilled portion of the bodied oil from the still as the improved drying oil.

4. The process of producing an improved drying oil which comprises in combination subjecting a bodied fish oil which fish oil in its unbodied condition had an iodine number about about 120, to high vacuum unobstructed path distillation until approximately 10% of the bodied fish oil has been distilled and then removing the undistilled portion of the bodied oil from the still as the improved drying oil.

5. The process of producing an improved drying oil which comprises in combination subjecting a bodied drying or semi-drying vegetable or animal oil to high vacuum unobstructed path distillation by causing it to flow in a thin film by centrifugal force over a heated vaporizing surface, applying the distillation treatment until approximately 2-12% of said bodied vegetable or animal oil has been distilled and then removing the undistilled portion of the bodied oil from the still as the improved drying oil.

6. The process of producing an improved drying oil which comprises in combination subjecting a bodied fish oil, which fish oil in its unbodied condition had an iodine number above about 120, to high vacuum unobstructed path distillation by causing it to flow in a thin film by centrifugal force over a heated rotating vaporizing surface, continuing the distillation treatment until approximately 2-12% of the bodied fish oil has been distilled and removing the un-

distilled portion of the bodied oil from the still as the improved drying oil.

7. The process of producing an improved drying oil which comprises in combination subjecting bodied menhaden oil to high vacuum unobstructed path distillation until approximately 10% of the bodied menhaden oil has been distilled and then removing the undistilled portion of the bodied oil from the still as the improved drying oil.

10

8. The process of producing an improved drying oil which comprises in combination subjecting bodied sardine oil to high vacuum unobstructed path distillation until approximately 5 10% of the bodied sardine oil has been distilled and then removing the undistilled portion of the bodied oil from the still as the improved drying oil.

RICHARD S. MORSE.